

Patented Jan. 12, 1926.

1,569,484

# UNITED STATES PATENT OFFICE.

EVERETT JOEL HALL, OF PASSAIC, NEW JERSEY, ASSIGNOR TO METALS DISINTEGRATING COMPANY, INC., OF NEW YORK, N. Y., A CORPORATION OF NEW YORK.

## PROCESS AND METHOD OF DISINTEGRATING METALS IN A BALL MILL OR THE LIKE.

No Drawing. Application filed March 25, 1919, Serial No. 285,055. Renewed June 3, 1925.

To all whom it may concern:

Be it known that I, EVERETT J. HALL, a citizen of the United States, residing at Passaic, in the county of Passaic and State 5 of New Jersey, have invented certain new and useful Improvements in Processes and Methods of Disintegrating Metals in a Ball Mill or the like, of which the following is a specification.

10 This invention relates to the reduction of metals to a finely divided condition in the nature of a dry powder or dust, in which the individual particles are in the form of minute relatively flat flakes, such as may be

15 used for the production of metal paint, etc. The practice of the invention may involve a preliminary disintegration of the metal, and then subjecting it to the mechanical action of steel balls or the like in an ordinary ball-mill, whereby disintegration is completed to the desired fineness.

20 One of the objects of the invention is to facilitate, in a mechanical sense, the breaking up of the particles of metal into smaller particles without relative loss of the 25 flat surface of the particle, and whereby the time and the power consumed in the disintegration are greatly reduced.

25 A further object is to conduct the disintegration aforesaid with the particles of the metal under treatment well covered with a liquid in the nature of an oil or its equivalent, this liquid having the property:—

30 (1) Of protecting the metal under treatment against the effects of atmosphere during the disintegration, as for instance oxidation, explosion and the like;

35 (2) Of lubricating the metal particles so that the reduction of them by the balls or other disintegrating means is more easily and quickly accomplished;

40 (3) Of forming with the metal particles, a mixture like a cream, sludge, or emulsion which is tenacious, cohesive and adhesive, and resistant to separation or segregation of its constituents and to the destruction of its own continuity, and which accordingly maintains a substantially uniform, continuous and homogeneous character during the 45 disintegration, a mixture in which the tendency of the metal particles to settle out is minimized;

50 (4) Of constituting a vehicle for the metal particles which will adhere evenly to the surfaces of the mill and of the balls by

means of which the reduction or disintegration is carried on, so that from the impact of ball against ball or ball against mill-wall at any point there will also result the flattening or reduction of a particle or particles 60 of metal carried in the oily sludge or cream which over-spreads the opposing surfaces, the sludge being of such consistency that it will coat the balls, but not so thick as to unduly cushion the blow of the balls when 65 they come together or strike the mill-wall;

(5) Of having a boiling point sufficiently high to prevent extensive loss by vaporization during the disintegrating process, but not so high that there will be difficulty in 70 removing it completely later on when the disintegration has been finished;

(6) Of being chemically inert, throughout the operation, to the metal under treatment, and preferably also non-inflammable; 75

(7) Of being easily removed by evaporation from the metal particles after disintegration is completed, but leaving the particles with a coating of grease.

Still another, and more specific, object of 80 the invention is to provide a protective vehicle or covering for the metal particles while they are in a ball-mill or the like and for the attainment of the object last-mentioned set forth, which comprises a large proportion of a relatively readily vaporizable oil, and a small proportion of a grease, having a 85 boiling point higher than that of the oil.

In the practical carrying out of the invention the metal, such as aluminum, if in 90 solid form, as a bar or the like, is first divided or reduced to a form from which the final reduction or comminution can more readily be carried on, as by turning it down in a lathe, whereby to produce chips or shavings of a size to facilitate further reduction. During this preliminary reduction the metal may be maintained entirely covered with a liquid as hereinafter described, a convenient way of accomplishing this being to immerse 95 the metal and cutter in a bath of the liquid. To insure that the liquid shall not reach boiling or decomposition temperature on account of the heat necessarily resulting from high-speed production, it may be continuously renewed, or initially supplied in sufficient 100 quantity. The final reduction is accomplished preferably in a ball-mill, in which the metal particles are subjected to the hammering action of ball against ball and ball 105 110

against mill-wall. During this operation the metal is kept well covered with a liquid having the properties above set forth. I have had good results with a mixture of varnoline (a petroleum fraction oil with a boiling point between 307° and 405° F), and stearine, in the proportion (assuming that there is 1.5 lb. of metal, as copper, under treatment) of 0.75 lb. of varnoline, 50.00 lb. of 5 balls, and stearine about 0.33% of the weight of copper. This liquid protects the metal against the effects of atmosphere, lubricates the particles so that their further reduction is facilitated, carries and supports the particles by reason of its creamy consistency, against the tendency of the particles to settle out and separate, and adheres evenly to the surfaces of the mill and of the balls, so that from the impact of ball against ball, or ball 10 against mill-wall at any point there will result the flattening or reduction of a particle or particles of metal carried in the oily vehicle which over-spreads the opposing surfaces. This liquid has a boiling point sufficiently high to prevent extensive loss by vaporization during the disintegrating process, but not so high that there will be difficulty in removing it completely later on when the disintegration has been finished. The 15 liquid is chemically inert to the metal under treatment and to the metal of the mill and the balls, and may if desired be rendered substantially non-inflammable by the addition of suitable chemicals, as for instance 20 carbon tetrachloride.

Upon completion of disintegration the contents of the mill are subjected to evaporation, preferably under conditions of vacuum, so that the varnoline goes off at a comparatively low temperature, thus minimizing the danger of the metal catching fire on removal from the dryer while hot. In the process of vacuum drying, of course, the distillate may be recovered for re-use. After the oil has all 40 gone off, the stearine remains in the shape of a coating on the particles. Such a coating is believed to be desirable where the powder is to be used for decorative purposes.

I prefer to use polished steel balls in the 45 milling operation, because I have found that roughened balls tend to break up the metal particles without flattening them to the desired extent.

It will be appreciated that as the disintegration of the metal proceeds, the total surface area of the metal particles is enormously increased and for that reason I may begin the disintegration with a sufficient amount of the liquid and add other additional quantities of varnoline or stearine, or both, at intervals as the disintegration goes on. And when the disintegration has been carried out to the desired extent I may add a considerable amount of the varnoline in 55 order to make the contents of the mill more

fluid and utilize the liquid as a vehicle for carrying the metal to the filter and/or dryer, where of course the oil is driven off and recovered for re-use.

In grinding the metal it is apt to become 70 warm due to the mechanical action, and if the liquid has not been rendered non-inflammable there will be a short interval of time when there is a possibility of explosion of the oil vapors, if there is access of atmosphere. To obviate the possibility of such an explosion I contemplate exhausting the air from the mill, its place being taken by the oil vapors which will be given off. Or of course a simple remedy will be to make the 75 liquid non-inflammable or to use a non-inflammable liquid in the first instance. Furthermore, I contemplate keeping down the temperature of the mill during operation by a spray of cooling water or the like. In the case of continuous grinding, that is, where the oil and metal are fed and discharged continuously and the oil returned after being separated from the metal, the temperature 80 may be maintained by some outside cooling means, or by circulation through pipes which are air cooled or water cooled, or any other desirable means. While this cooling is not strictly essential to operation, it does undoubtedly lessen the risk of fire in 85 the case of inflammable liquids, and prevents loss of liquid from evaporation whether the liquid is inflammable or non-inflammable. 90

I claim:

1. The art of manufacturing metal dust 100 which consists in mechanically disintegrating the metal, while keeping it covered with a lubricating liquid which protects the metal against the effects of atmosphere and is inert to the metal, and which has a boiling point high enough to prevent excessive loss by vaporization during the disintegration, but not so high that there will be difficulty in its separation later from the metal by vaporization; and thereafter freeing the 105 disintegrated material from the liquid by evaporation of the liquid, to produce a dry metallic powder.

2. The art of manufacturing finely divided metal in the form of minute relatively 110 flat flakes, which consists in subjecting the metal to the action of a ball mill or the like, while keeping it covered with a lubricating liquid which protects the metal against the 115 effects of atmosphere and is inert to the metal, and which has a boiling point high enough to prevent excessive loss by vaporization during the disintegration, but not so high that there will be difficulty in its separation later from the metal by vaporization; and thereafter evaporating the liquid from 120 around and between the particles to produce a dry metallic powder.

3. The art of manufacturing finely divided metal in the form of minute relatively 125

flat flakes, which consists in subjecting the metal to the action of a ball mill or the like, while keeping it covered with a lubricating liquid which protects the metal against the 5 effects of atmosphere and is inert to the metal, and which has a boiling point high enough to prevent excessive loss by vaporization during the disintegration, but not so high that there will be difficulty in its separation 10 later from the metal by vaporization, preventing decomposition of the liquid during the disintegration, and thereafter evaporating the liquid from around and between the particles to produce a dry metallic powder.

4. As a step of the process of disintegrating metals in a ball-mill or the like, keeping the metal under treatment covered with a liquid consisting of a plurality of ingredients 20 having a definite boiling point which forms with the metal particles, in the operation of the mill, a homogeneous mixture like a thick cream, sludge or emulsion which is tenacious, cohesive and adhesive and resistant to separation or segregation of its constituents and to the destruction of its own continuity and which maintains a substantially uniform, continuous and homogeneous character during the disintegration.

5. The method of disintegrating metal in a ball mill or the like which comprises keeping the metal well covered with a liquid comprising a large proportion of a relatively 30 readily vaporizable oil, and a small proportion of a grease having a boiling point higher than that of the oil, and when the disintegration is completed, driving off from the metal particles the readily vaporizable oil without disturbing the grease.

6. As a step in the process of disintegrating metals in a ball-mill or the like, keeping the metal particles well covered with a liquid chemically inert to the metal and having a boiling point sufficiently high to prevent extensive loss by evaporation during the disintegrating process, but not so high that there 40 will be difficulty in removing it completely

later on when the disintegration has been finished, such liquid having the property of forming with the metal particles a homogeneous mixture like a cream, sludge, or emulsion which is tenacious, cohesive, and resistant to separation or segregation of its constituents and to the destruction of its own continuity and which maintains a substantially uniform continuous and homogeneous character, adhering evenly to the surfaces of the mill and of the balls by means of which the reduction or disintegration is carried on, so that from the impact of ball against ball or ball against mill-wall at any point there will result the flattening or reduction of a particle or particles of metal carried in the sludge which over-spreads the opposing surfaces, the sludge being of such consistency that it will coat the balls, but not so thick as to unduly cushion the blow of the balls when they come together or strike the mill-wall; and effecting separation of the metal particles from the liquid 50 after the disintegration has been completed, to leave the metal particles in a substantially dry state.

7. The method of disintegrating metals, consisting of the steps set forth in claim 3 55 with the additional step of adding a sufficient amount of oil to the contents of the mill when the disintegration is completed necessary for carrying the metal particles out of the mill.

8. The process of manufacturing metal powder which consists in mechanically disintegrating metal, while keeping it covered with a lubricating liquid which protects the metal against the effects of atmosphere and 60 is inert to the metal, and which has a boiling point high enough to prevent excessive loss by vaporization during the disintegration, but not so high that there will be difficulty in its separation later from the 65 metal by vaporization.

In testimony whereof I affix my signature.

EVERETT JOEL HALL.